

March 28, 1944.

C. M. CROFT ET AL

2,344,973

DYEING CELLULOSE DERIVATIVES

Filed March 19, 1941



C. M. CROFT  
W. H. HINDLE

INVENTORS

BY  
*J. Belter & Co., Inc.*  
ATTORNEYS

## UNITED STATES PATENT OFFICE

2,344,973

## DYEING CELLULOSE DERIVATIVES

Cyril M. Croft and Walter H. Hindle, Cumberland, Md., assignors to Celanese Corporation of America, a corporation of Delaware

Application March 19, 1941, Serial No. 384,058

14 Claims. (Cl. 8—59)

This invention relates to the dyeing of organic derivative of cellulose textile materials and relates more particularly to the dyeing of organic derivative of cellulose textile materials by mechanical impregnation methods.

An object of our invention is to increase the speed of dyeing of organic derivative of cellulose textile materials.

Another object of our invention is to obtain more uniform dyeings of organic derivative of cellulose textile materials and to obtain said dyeings more economically.

Other objects of our invention will appear from the following detailed description and the accompanying drawing.

The drawing shows diagrammatically a side elevation of a padding device, one form of apparatus by which our invention may be practiced.

In the coloration of textile materials by means of dye baths it is highly desirable that the depth of shade desired in the textile material be reached with as short an immersion time and as little handling of the material as possible. When dyeing organic derivative of cellulose textile materials, however, it has been found that these materials are dyed more slowly than other textile materials since they are less absorbent and the dye liquor in the dye bath does not penetrate them as rapidly or as completely as other textile material. Many dyestuffs when applied to organic derivative of cellulose material from aqueous baths yield dyeings which are far from satisfactory and consequently long periods of immersion and manipulation are usually required in order to dye the textile materials in sufficiently deep, non-fugitive shades.

We have now discovered that organic derivative of cellulose textile materials may be dyed rapidly in deep, uniform, level shades with dyestuffs normally having little or no affinity for organic derivatives of cellulose and relatively water insoluble dyestuffs which are usually applied in dispersed or solubilized form, if said dyestuffs are dissolved in an organic liquid medium comprising at least 70% by weight of a lower aliphatic alcohol, and the resulting dye solution applied to the textile material by mechanical impregnation methods. Substantial increases in the rate of production are made possible and satisfactory dyeings may be obtained with a minimum manipulation of the materials and a low concentration of dyestuffs in the dye bath.

The lower aliphatic alcohols which are suitable for use in the dye bath may be those alcohols which are solvents for the dyestuffs em-

ployed and which exert at least a swelling or softening action on the organic derivatives of cellulose. While we prefer to employ ethyl alcohol in the dye liquor, other alcohols such as methyl alcohol, propyl alcohol, isopropyl alcohol, n-butyl alcohol, secondary butyl alcohol, tertiary butyl alcohol, n-amyl alcohol, secondary amyl alcohol and tertiary amyl alcohol, or mixtures of these alcohols may be used. The amount of the alcohol used in the dye liquor will vary depending upon the alcohol or alcohols used, but should comprise at least 70%, by weight, of the dye bath. Where ethyl alcohol is being used the dye liquor should preferably contain from about 75 to 80% by weight of the alcohol.

Various dyestuffs may be employed. These dyestuffs may be acid dyes which are used for the dyeing of wool and normally show little or no affinity for organic derivatives of cellulose, or they may be those dyes which are relatively insoluble in water and which are applied to organic derivative of cellulose materials in the form of aqueous dispersions after being specially solubilized. When these dyestuffs are applied to organic derivative of cellulose textile materials by mechanical impregnation methods in alcoholic solutions in accordance with our process, the resulting dyeings are of uniform depth and brilliance and may be obtained with relatively short immersion times. The amount of the dyestuff dissolved in the dye liquor will vary depending upon the final shade desired in the material which is being dyed and may be from as low as 0.01% up to 4.0%, based on the weight of the material to be dyed.

The dye liquor may be applied to the organic derivative of cellulose textile materials by padding, spraying or by other convenient method of mechanical impregnation. Thus, as a continuous process, a fabric may be unwound from a roll, passed through a solution of the dyestuff, then between nipping rolls of a padding mangle which are adjusted to permit the desired amount of dye liquor to be retained in the fabric, and the fabric then subjected to rapid drying. The period of immersion of the fabric in the dye liquor is relatively short and may be from 1½ to 10 seconds. If desired, the fabric may be processed through the padding mangle at speeds ranging up to 45 yards per minute.

Not only is our process applicable to the dyeing of fabrics, but especially desirable results are obtained when organic derivative of cellulose staple fiber in the form of a top is dyed in this way. Not only may more uniform dyeings be obtained but

increased production may be achieved along with a reduction in the amount of dyestuff necessary in order to obtain a desired shade. By carrying out the dyeing operation in accordance with my invention, the required shade for the material may be obtained by test samples prior to running the material through the dye bath, thereby eliminating the necessity for adding additional color while the fabric or top is dyeing. The level of liquid in the dye bath is maintained by the addition thereto from time to time of dye liquor of the same composition as that initially employed to replace that portion of the dye liquor carried out by the fabric. Consequently, there is no need to drop incompletely exhausted dye baths when the final shade is obtained as in conventional methods of dyeing, and this source of loss or waste of color is eliminated. When dyeing staple fibers in the form of a top, a large number of ends may be run through the dye bath at the same time and padded by a single pad, thus greatly increasing the rate of production of dyed staple without additional equipment. The time of immersion of the top in the dye liquor prior to padding may be from 1½ seconds to 2 minutes. After padding, the dyed top is subjected to rapid drying.

The dyed textile materials in the form of fabrics or tops may be dried by passing said materials through a chamber through which there is circulated air heated to temperatures up to about 95° C. for quite rapid drying and heated to say 70° C. to 90° C. for less rapid drying. Where the particular solvent mixture used exerts a marked swelling action on the organic derivatives of cellulose it is advantageous that the materials be dried rapidly. While drying by means of heated air is preferable, heated drums or cans may also be used.

The organic derivative of cellulose fabrics, tops, yarns or other textile materials which may be dyed in accordance with our process may be cellulose esters or cellulose ethers. Examples of cellulose esters are cellulose acetate, cellulose propionate, cellulose butyrate, and mixed esters such as cellulose acetate-propionate and cellulose acetate-butyrate, while examples of cellulose ethers are ethyl cellulose and benzyl cellulose. The materials may be mixed materials containing organic derivatives of cellulose and yarns or fibers of other materials such as cotton, silk, wool or regenerated cellulose and in this way differential dyeings may be obtained where the dyes used have no affinity for the other textile materials present. Especially valuable differential dyeings or cross-dyed effects may be obtained on fabrics containing mixed cellulose acetate and wool yarns when specially solubilized, dispersed dyes of the "SRA" type are used. The cellulose acetate fibers may be dyed fairly heavy shades while the wool fibers remain uncolored and unstained. If desired, the wool fibers may later be dyed with dyestuffs which have affinity for the wool or the wool may be left uncolored.

As an aid in describing our invention, the same will be described with reference to the accompanying drawing wherein there is shown a padding device, which also constitutes part of our invention. The device, as shown, comprises a dye trough 1 containing the dye liquor 2, the dye trough being provided with a freely rotatable roller 3 mounted therein, the roller being adapted to act as a fabric guide. Positioned near the dye trough 1 is a padding mangle comprising a plu-

rality of rolls 4, 5 and 6, which are suitably driven for continuous rotation. While a three roll pad mangle is shown in the drawing, a two roll pad mangle may be employed if desired. The nip or distance between said rolls may be adjusted as desired in accordance with the type of material being processed and the quantity of liquor which is to be permitted to remain thereon. The fabric 7 which is being dyed, may be drawn from a roll 8 wound about a suitable core 9 which is mounted so as to be freely rotatable. The fabric is passed over guide rolls 10 and 11 and is then passed into the dye liquor under roller 3. The fabric carrying the dye liquor is then passed over an expander bar 12 and into the nip of rolls 4 and 5 which is so adjusted as to permit the fabric 7 to retain the desired amount of dye liquor thereon. The dye liquor expressed from the fabric is caught by means of a suitable trough (not shown) placed below the rolls of the padding mangle. After passing through the nip of rolls 4 and 5, the fabric 7 is passed over another expander bar 13 and through the nip of rolls 5 and 6, after which it passes over guide rollers 14 and 15 and enters a tall heated chamber 16 where the dye solvent is removed by heated air circulated by means of a hot air blower 17. When a two roll pad mangle is used, only a single expander bar need be employed. The use of expander bars in connection with this pad dyeing device both before and after the wet fabric enters the nip of the padding mangle overcomes any difficulties experienced in processing the fabric due to creasing or to shrinkage in the dye bath and comprises a novel advance in the art. It will of course be understood that the method of immersion of the fabric in the dye liquor may be varied. In lieu of merely passing the fabric under a roll, the fabric may be passed through the nip of a pair of rolls submerged in the dye bath or else the fabric may first be dipped and then nipped between submerged rolls. Likewise, where it is desired to maintain the fabric in the dye bath for longer periods of time the bath may be made long and relatively shallow and the submerged fabric run through the bath at any desired speed. In this way the fabric may be kept immersed for any desired period.

In order further to illustrate our invention but without being limited thereto, the following examples are given:

#### Example I

A dye bath having the following composition is made up:

|                                                                                          | Parts by weight |
|------------------------------------------------------------------------------------------|-----------------|
| Celliton Fast Blue AF (1-methylamino-4-isopropyl - amino-2-carboxyamide - anthraquinone) | 31.0            |
| SRA Red VIII (p-nitroaniline-azo-dioxyethyl-m-toluidine)                                 | 2.5             |
| SRA Orange BL (2-chlor-4-nitro-6-brombenzene - azo-dioxyethyl-m-chlor aniline)           | 2.0             |
| Ethyl alcohol                                                                            | 6300            |
| Water                                                                                    | 2000            |

A cellulose acetate fabric of a satin weave is passed into a dye bath or trough containing the above dye liquor and beneath a roller submerged therein, as heretofore described, the dye liquor being maintained at a temperature of 20° to 25° C. and at a suitable level. The fabric is passed continuously through the dye bath, at the rate of 10 yards per minute, the arrangement being

such that the fabric is immersed in the dye liquor for 6 seconds. The fabric laden with dye liquor is then passed over an expander bar, through the lower nip of a padding mangle, over a second expander bar and finally through the upper nip of the padding mangle. The nip of the rolls is so adjusted that the fabric retains 65% of its own weight of the dye liquor. From the nip of padding mangle the fabric is passed into a drying chamber in which air heated to 95° C. is circulated. After being dried, the fabric is scoured, tenered and calendered. The fabric thus dyed is a deep clear blue. The entire operation may be carried out in a matter of 30 to 60 minutes, whereas the usual dyeing process required from 4 to 8 hours for the same results on an equivalent quantity of fabric.

#### Example II

A mixed cellulose acetate and wool fabric containing 80% of cellulose acetate and 20% of wool is dyed by passing it through a dye liquor having the same composition as the dye liquor in Example I. The fabric is maintained in the dye bath for 6 seconds and the fabric laden with the dye liquor is then passed between the double nip of the padding mangle. The rolls are so spaced that about 70% on the weight of the fabric of dye liquor is retained by the fabric. The fabric from the padding mangle is passed to a drying chamber in which air heated to about 95° C. is circulated. After being dried, the fabric is washed for 10 minutes at 20° C. in a solution containing 5 grams per liter of a suitable fatty alcohol sulfate detergent such as "Gardinol WA," and then rinsed in cold water. The fabric is then washed again for 10 minutes at 60° C. with additional detergent solution of the same composition. The scouring or washing is carried out to remove excess dyestuff before the dyeing of the wool is undertaken. The undyed wool of the mixed material remains clean and unstained while the cellulose acetate fibers are dyed a deep blue.

#### Example III

A dye liquor having the following composition is prepared:

|                                                    | Parts by weight |
|----------------------------------------------------|-----------------|
| SRA Orange BL                                      | 290             |
| SRA Golden Yellow XI (dinitro-amino-diphenylamine) | 1,125           |
| Celliton Fast Blue AF                              | 3,000           |
| Ethyl alcohol                                      | 240,000         |
| Water                                              | 80,000          |

Cellulose acetate staple fiber in the form of a loose top is entered into this dye liquor which is at a temperature of 20° to 25° C. and the top is passed through the bath in such a manner that it remains immersed therein for 2 minutes. On leaving the dye bath the top is run through the rolls of the padding mangle at about 10 yards per minute and 60% of dye liquor is permitted to remain in the top as it enters the drying chamber in which air heated to 95° C. is circulated. After drying, the top is rinsed to remove any surface color and alcoholic odor and is again dried, the whole dyeing operation taking place in 15 to 30 minutes. Not only does the dyeing by means of an alcoholic dye liquor thus enable the top to be dyed with unusual speed, but the top may be handled freely during the entire operation for the alcoholic dye liquor serves to give the top a surprisingly increased wet strength.

#### Example IV

A dye liquor having the following composition is prepared:

|                                           | Parts by weight |
|-------------------------------------------|-----------------|
| 5 Amacid Black BR Supra (acid dye)        | 500             |
| Xylene Milling Blue GL (color index #833) | 250             |
| Ethyl alcohol                             | 60,000          |
| Water                                     | 20,000          |

A cellulose acetate fabric is passed into a trough or dye bath containing the above dye liquor and beneath a roller, as heretofore described, the dye liquor being maintained at a temperature of 20° to 25° C. and at a suitable level. The dyeing of the fabric is carried out in a manner analogous to Example I and the fabric is thus dyed a navy blue.

It is to be understood that the foregoing detailed description is given merely by way of illustration and that many variations may be made therein without departing from the spirit of our invention.

Having described our invention, what we desire to secure by Letters Patent is:

1. Method for the coloration of an organic derivative of cellulose textile material which comprises padding such a textile material with an aqueous alcoholic solution of a dyestuff, said aqueous alcoholic solution comprising at least 70%, by weight, of a lower aliphatic alcohol which is a solvent for the dye, and then rapidly drying said material at an elevated temperature.

2. Method for the coloration of a cellulose acetate textile material which comprises padding such cellulose acetate textile material with an aqueous alcoholic solution of a dyestuff, said aqueous alcoholic solution comprising at least 70%, by weight, of a lower aliphatic alcohol which is a solvent for the dye, and then rapidly drying said material at an elevated temperature.

3. Method for the coloration of a cellulose acetate textile material which comprises padding such cellulose acetate textile material with an aqueous alcoholic solution of a dyestuff, said aqueous alcoholic solution comprising at least 70%, by weight, of ethyl alcohol and then rapidly drying said material at an elevated temperature.

4. Method for the coloration of a fabric containing yarns of an organic derivative of cellulose which comprises padding the fabric with an aqueous alcoholic solution of a dyestuff, said aqueous alcoholic solution comprising at least 70%, by weight, of a lower aliphatic alcohol which is a solvent for the dye, and then rapidly drying said fabric at an elevated temperature.

5. Method for the coloration of a fabric containing yarns of cellulose acetate which comprises padding the fabric with an aqueous alcoholic solution of a dyestuff, said aqueous alcoholic solution comprising at least 70%, by weight, of a lower aliphatic alcohol which is a solvent for the dye, and then rapidly drying said fabric at an elevated temperature.

6. Method for the coloration of a fabric containing yarns of cellulose acetate which comprises padding the fabric with an aqueous alcoholic solution of a dyestuff, said aqueous alcoholic solution comprising 75%, by weight, of ethyl alcohol and 25%, by weight, of water, and then rapidly drying said fabric at an elevated temperature.

7. Method for the coloration of organic derivative of cellulose filaments associated together in the form of a top which comprises padding such

a top with an aqueous alcoholic solution of a dyestuff, said aqueous alcoholic solution comprising at least 70%, by weight, of a lower aliphatic alcohol which is a solvent for the dye, and then rapidly drying said top at an elevated temperature.

8. Method for the coloration of cellulose acetate filaments associated together in the form of a top which comprises padding said cellulose acetate top with an aqueous alcoholic solution of a dyestuff, said aqueous alcoholic solution comprising at least 70%, by weight, of a lower aliphatic alcohol which is a solvent for the dye, and then rapidly drying said top at an elevated temperature. 10

9. Method for the coloration of cellulose acetate filaments associated together in the form of a top which comprises padding said cellulose acetate top with an aqueous alcoholic solution of a dyestuff, said aqueous alcoholic solution comprising at least 70%, by weight, of ethyl alcohol, and then rapidly drying said top at an elevated temperature. 20

10. Method for the coloration of cellulose acetate filaments associated together in the form of a top which comprises padding said cellulose acetate top with an aqueous alcoholic solution of a dyestuff, said aqueous alcoholic solution comprising 75%, by weight, of ethyl alcohol and 25%, by weight, of water, and then rapidly drying said top. 25

11. Method for the coloration of organic derivative of cellulose fibers in a textile material containing fibers of an organic derivative of cellulose and other fibers, which comprises padding said textile material with an aqueous alcoholic

solution of a dyestuff, said aqueous alcoholic solution comprising at least 70%, by weight, of a lower aliphatic alcohol which is a solvent for the dye, and then rapidly drying said material at an elevated temperature. 5

12. Method for the coloration of the organic derivative of cellulose fibers in a textile material containing fibers of an organic derivative of cellulose and animal fibers which comprises padding said textile material with an aqueous alcoholic solution of a dyestuff, said aqueous alcoholic solution comprising at least 70%, by weight, of a lower aliphatic alcohol which is a solvent for the dye, and then rapidly drying said material at an elevated temperature. 10

13. Method for the coloration of the cellulose acetate in a textile material containing fibers of cellulose acetate and wool fibers which comprises padding said textile material with an aqueous alcoholic solution of a dyestuff, said aqueous alcoholic solution comprising at least 70%, by weight, of a lower aliphatic alcohol which is a solvent for the dye, and then rapidly drying said material at an elevated temperature. 20

14. Method for the coloration of the cellulose acetate in a textile material containing fibers of cellulose acetate and wool fibers which comprises padding said textile material with an aqueous alcoholic solution of a dyestuff, said aqueous alcoholic solution comprising 75%, by weight, of ethyl alcohol and 25%, by weight, of water, and then rapidly drying said material at an elevated temperature. 25

CYRIL M. CROFT.  
WALTER H. HINDLE.